# EUROPEAN PATENT SPECIFICATION

(11) **EP 1 623 060 B1**
(45) Date of publication and mention of the grant of the patent: **09.05.2007**
(21) Application number: 04733135.0
(22) Date of filing: 14.05.2004
(51) Int. Cl.: D01F 1/02, D01F 1/04, D01F 1/10

(54) **METHOD OF MAKING LASER-MARKABLE FIBERS OR FIBER PRODUCTS**
VERFAHREN ZUR HERSTELLUNG VON LASERBESCHRIFTBARE FASERN ODER FASERPRODUKTE
METHODE POUR LA PREPARATION DE FIBRES OU PRODUITS DE FIBRES MARQUABLES AU LASER

(30) Priority: 14.05.2003 JP 2003136426
(43) Date of publication of application: 08.02.2006
(73) Proprietor: Shikibo Ltd., Osaka-shi, Osaka 541-8516 (JP); Clariant Finance (BVI) Limited, Road Town, Tortola (VG)
(72) Inventor: TSUJIMOTO, Yutaka, Akashi-shi, Hyogo 6730011 (JP); SAKAI, Yoshiaki, Kashihara-shi, Nara 6340051 (JP); LOYRION, Frédéric, c/oClariant (France), F-78205 Mantes-la-Jolie, Cedex (FR)
(74) Representative: Müller-Boré & Partner Patentanwälte
(86) International application number: PCT/JP2004/006864
(87) International publication number: WO 2004/101870

(56) References cited:
- WO-A1-94/29499
- WO-A1-98/03708
- DE-A1- 4 431 735
- DE-A1- 10 118 704
- JP-A- 63 227 828
- US-A- 5 697 390
- US-B1- 6 482 511
- PATENT ABSTRACTS OF JAPAN vol. 1998, no. 10, 31 August 1998 (1998-08-31) & JP 10 121328 A (UNITIKA LTD), 12 May 1998 (1998-05-12)
- PATENT ABSTRACTS OF JAPAN vol. 1998, no. 09, 31 July 1998 (1998-07-31) & JP 10 088428 A (NIPPON ESTER CO LTD), 7 April 1998 (1998-04-07)
- PATENT ABSTRACTS OF JAPAN vol. 1997, no. 11, 28 November 1997 (1997-11-28) & JP 09 195125 A (MITSUBISHI RAYON CO LTD), 29 July 1997 (1997-07-29)
- PATENT ABSTRACTS OF JAPAN vol. 1997, no. 07, 31 July 1997 (1997-07-31) & JP 09 077961 A (NIPPON ESTER CO LTD), 25 March 1997 (1997-03-25)
- PATENT ABSTRACTS OF JAPAN vol. 017, no. 225 (C-1055), 10 May 1993 (1993-05-10) & JP 04 361608 A (KANEBO LTD), 15 December 1992 (1992-12-15)
- PATENT ABSTRACTS OF JAPAN vol. 016, no. 298 (C-0958), 2 July 1992 (1992-07-02) & JP 04 082910 A (SHINKASHIYOU:KK), 16 March 1992 (1992-03-16)

## Description

### TECHNICAL FIELD

The present invention relates to a method of making a laser-markable fiber or fiber product.

### BACKGROUND ART

Methods generally used for marking a fiber or fiber product with a pattern or a mark such as a letter or symbol include printing the fiber or fiber product using a dye, pigment or the like; and printing on the fiber or fiber product using an inkjet printer, etc. (see, for example, Japanese Unexamined Patent Publications Nos. 1990-41480 and 1995-336466 or US-A-6 482 511).

Further, synthetic polymers comprising carbon black and barium sulfate are described in DE-A-10 118 704.

However, the above methods can not be used to produce minute marks such as letters or symbols on fibers or fiber products. Therefore, it has been impossible to mark individual yarns with such marks.

### DISCLOSURE OF THE INVENTION

An object of the invention is to provide a method of making a fiber or fiber product wherein the individual yarns can be marked with minute marks. In this specification, "individual yarns" include spun yarns, monofilament yarns, multifilament yarns and composite yarns thereof.

The present inventors carried out intensive research to develop a method of making a fiber or fiber product wherein the individual yarns can be marked with a minute mark, such as letters or symbols. As a result, the inventors found that a fiber or fiber product that achieves the above object can be produced by kneading into an artificial fiber a filler whose own color changes or a filler mixture whose entire color appears to change by irradiation with a laser beam. The present invention has been accomplished based on this finding.

The invention provides the following methods:
1. A method of marking a fiber or fiber product with a mark or pattern, comprising irradiating with a laser beam a fiber or fiber product prepared by impregnating an artificial fiber with carbon black and barium sulfate, so that the irradiation causes phase separation of carbon black and allows barium sulfate to clearly appear on the surface of the fiber or fiber product, thereby changing the laser beam-irradiated portion from black to white.
2. The method according to claim 1, wherein the artificial fiber is a polyester.

### Fibers or fiber products obtainable with the methods of the invention

The fiber or fiber product provided by the invention comprises an artificial fiber and a filler incorporated therein. The filler is a filler mixture of carbon black and barium sulfate whose entire color appears to change by irradiation with a laser beam.

Any of a wide variety of known artificial fibers can be used as the artificial fiber so long as a filler whose own color changes or a filler mixture whose entire color appears to change by irradiation with a laser beam can be incorporated thereinto. Examples of such artificial fibers include synthetic fibers, semi-synthetic fibers, regenerated fibers, and inorganic fibers.

Examples of usable synthetic fibers include polyesters, aliphatic polyamides, aromatic polyamides, polyethylenes, polypropylenes, vinylons, acrylics, polyvinyl alcohols, polyurethanes and the like.

Examples of usable semi-synthetic fibers include acetates, triacetates, promix and the like.

Examples of usable regenerated fibers include rayon, cupra and the like.

Examples of usable inorganic fibers include carbon fibers, ceramic fibers and the like.

Among the artificial fibers, synthetic fibers are preferable, and polyesters are more preferable. Specific examples of polyesters include polyethylene terephthalate, polytrimethylene terephthalate, polytetramethylene terephthalate and the like.

Examples of artificial fibers include slit yarns produced by slitting a plastic film such as polyethylene terephthalate, polyethylene or polypropylene. Such slit yarns usually have a width of about 0.1 to about 0.8 mm, and preferably about 0.15 to about 0.37 mm; and usually have a thickness of about 20 µm or less, and preferably about 2 to about 12 µm.

The artificial fibers may be used singly or spun, plied or twisted together.

The artificial fibers may have a core-sheath structure. Examples of artificial fibers with a core-sheath structure include those produced by using a slit yarn as a core and winding another fiber (spun yarn or filament yarn) therearound, those produced by using a spun yarn or filament yarn as a core and winding a slit yarn therearound and those comprising a monofilament yarn with an internal core-sheath structure.

The artificial fibers may have a uniform or nonuniform thickness. The cross section of artificial fibers may have any shape such as circular, elliptical, Y-shaped, cross-shaped, W-shaped, L-shaped, T-shaped, hollow, triangular, flat, star-shaped, cocooned, eight-leaved, dog-bone shaped (or dumbbell), etc.

The fiber includes not only these fibers but also primary processed products thereof, such as yarns, knits, woven fabrics, knitted fabrics, and nonwoven fabrics.

The artificial fiber may be a blend fabric blended with natural fibers such as cellulose fibers, animal hair fibers, and silks.

In this specification, a "fiber product" refers to a product obtained by further processing of a fiber. Examples of such products include outer garments, intermediate garments, innerwear and like clothing, beds and bedroom accessories, and interior accessories. Specific examples of fiber products include clothing such as coats, jackets, trousers, skirts, shirts, knitted shirts, blouses, sweaters, cardigans, nightwear, underwear, supporters, socks, tights, hats, scarves, mufflers, gloves, garment linings, garment stiffeners, cotton stuffing for clothes, work clothing, sanitary gowns, uniforms, prison uniforms, and schoolchildren's uniforms; beds and bedroom accessories such as mattress coverings, wadding cotton, pillow cases, sheets and the like; interior accessories such as curtains, mats, carpets, cushions, stuffed toys and the like; fancy goods such as towels, and handkerchieves ; yarn products such as machine sewing threads, embroidery threads, plaited cords, straps, braids, fishing lines and artificial baits; tags on merchandise; paper products or nonwoven fabrics; bags; materials for electronic products and construction materials.

Specific examples of paper products include securities such as stocks, national bonds, local bonds, gift vouchers, drafts, checks, postage stamps, revenue stamps, certificate stamps and admission tickets; vouchers such as coupons and public lottery tickets; paper currency; and various kinds of certificate forms.

Examples of the filler whose own color changes by irradiation with a laser beam is a mixture of carbon black and barium sulfate (BaSO₄).

The filler is preferably in the form of particles. The mean particle diameter is usually not more than about 15 µm, and preferably not more than about 1 µm. The particle diameter can be measured by, for example, laser diffraction methods.

The mean particle diameter of the white pigment barium sulfate is usually selected from a wide range of 10 nm to 3 µm, and preferably about 10 nm to about 1 µm.

The white pigment barium sulfate is usually used in an amount of 5 to 90 wt.%, and preferably about 10 to about 70 wt.%, relative to the weight of filler whose own color changes by irradiation with a laser beam.

Examples of carbon blacks include acetylene black, lamp black, thermal black, furnace black, channel black, and Ketjenblack, graphite, titanium black, and black iron oxide. Among these, carbon blacks are preferable in view of dispersibility and cost. Such black pigments can be used singly or in combination of two or more. Carbon blacks can be classified into acetylene black, oil black, gas black, etc. according to the raw materials, and any carbon black can be used.

The mean particle diameter of the carbon black (black pigment) is usually selected from a wide range of 10 nm to 3 µm, and preferably about 10 nm to about 1 µm It is preferable to have a mean particle diameter of 10 to about 30 nm.

The amount of carbon black (black pigment) is usually in the range of 0.1 to 80 wt.%, and preferably about 10 to about 50 wt.%, relative to the weight of the white filler barium sulfate.

The filler mixture whose entire color appears to change by irradiation with a laser beam is usually contained in the fiber or fiber product of the invention in an amount of 0.01 to 10 wt.%, preferably about 0.3 to about 3 wt.%, and more preferably about 0.6 to about 1.2 wt.%, relative to the total weight of artificial fiber and filler.

The fiber or fiber product may optionally contain other components such as known antimicrobial agents, UV absorbers, UV reflectors, colored (i.e., non-black, non-white) and pigments.

### Method of producing the fiber or fiber product of the invention

The fiber of the invention comprising a filler mixture whose entire color appears to change by irradiation with a laser beam can be produced by kneading the filler into the fiber during the process of spinning the fiber raw material into a fiber. When the artificial fiber has a core-sheath structure, the filler may be kneaded into either or both its core and sheath.

The fiber is produced, for example, by mixing and dispersing in a melt or solution of the artificial fiber raw material a filler mixture whose entire color appears to change by irradiation with a laser beam, and then spinning the resulting dispersion into a fiber. The filler is preferably mixed and dispersed in the fiber raw material in the form of a masterbatch.

A wide variety of known spinning methods such as melt-spinning methods, dry-spinning methods and wet-spinning methods can be used as the spinning method. Which spinning method is used depends on the kind of fiber raw material used.

When the fiber raw material can be melted in a thermally and chemically stable manner, it is preferable to use melt-spinning. In this case, a predetermined amount of filler may be mixed and dispersed in the melt of the fiber raw material. The fiber can be produced by ejecting the fiber raw material melt with a filler mixed and dispersed therein through a fine nozzle into the air, followed by air cooling and solidifying the molten filament while attenuating and then drawing it out at a constant speed. Fibers suited to melt-spinning are, for example, polyesters, aliphatic polyamides, polyethylenes and polypropylenes.

When the fiber raw material is stable at high temperatures and can dissolve in a volatile solvent, it is preferable to use dry-spinning. In this case, a predetermined amount of filler may be mixed and dispersed in a volatile solvent solution of the fiber raw material. The fiber can be produced by ejecting the fiber raw material solution with a filler mixed and dispersed therein through a fine nozzle into a heated gas and then solidifying the solution into a fiber while evaporating the volatile solvent. Fibers suited to dry-spinning are acrylics, and acetates.

When the fiber raw material dissolves only in low volatility solvents or solvents unstable at high temperatures, it is preferable to use wet-spinning. In this case, a predetermined amount of filler may be mixed and dispersed in a solution of the fiber raw material. The fiber can be produced by ejecting the fiber raw material solution with a filler mixed and dispersed therein through a fine nozzle into a coagulation bath containing a nonsolvent, and then solidifying it into a fiber while removing the solvent. Fibers suited to wet-spinning are, for example, polyvinyl alcohols and rayon.

When the fiber is in the form of slit yarns, it can be produced by slitting the following plastic films or multi-layered films using a cutter such as a micro slitter, tape slitter, etc.: a plastic film (e.g., polyethylene terephthalate, polyethylene, polypropylene, etc.) into which a filler mixture whose entire color appears to change by irradiation with a laser beam has been incorporated; a plastic film (e.g., polyethylene terephthalate, polyethylene, polypropylene, etc.) coated with a composition comprising a filler mixture whose entire color appears to change by irradiation with a laser beam; or multi-layered films produced by laminating other film(s) (e.g., polyethylene terephthalate) on the above plastic films.

Using a fiber produced by the above method, a fiber product can be produced by known methods such as sewing.

When the fiber product is a paper product, the paper product can be produced by scooping up the fiber produced by the above methods with a fine mesh screen.

Fibers or fiber products may be dyed using dyes or pigments appropriate to the fiber raw material.

### Method of using the fiber or fiber product obtainable with the methods of the invention

When the fiber or fiber product is impregnated with a filler mixture that changes color by irradiation with a laser beam is irradiated with a laser, the filler mixture changes color by laser beam irradiation. Therefore, it is possible to change the color of the fiber or fiber product only in the laser beam-irradiated portions. Phase separation or other phenomena occur in the filler mixture and the white pigment barium sulfate displays itself on the surface of the fiber or fiber product. As a result, it is possible to change the color of the fiber or fiber product only in the laser beam-irradiated portions.

Lasers usable for the invention are YAG lasers, excimer lasers, CO₂ lasers and the like. Of these lasers, YAG lasers are preferable, and Nd-YAG lasers are more preferable.

There is no limitation on the wavelength of the laser so long as it changes the color of the filler. In the case of Nd-YAG lasers, it is preferable that the wavelength be about 354 nm, about 532 nm or about 1064 nm.

The fiber or fiber product can be irradiated, for example, by using a scanning laser marking device. Since the laser beam irradiation can be controlled by computer, a minute distinguishing mark (e.g., logos, code numbers, serial numbers, etc.) can be produced in a predetermined position on the fiber or fiber product.

Slit yarn marked with a mark or pattern can be used as an anti-counterfeiting thread for paper products such as those mentioned above. "Thread" as used herein includes ribbons of film or foil, wires and any other suitable elongate elements for inclusion in paper products.

Therefore, by checking for the presence of a mark or pattern marked on the fiber or fiber product, it can be distinguished whether the fiber or fiber product is marked or unmarked.

More specifically, the fiber or fiber product is irradiated with a laser beam to produce a fiber or fiber product with a mark or pattern thereon. Marketed fibers or fiber products can then be checked for the presence of the mark or pattern to distinguish whether the fibers or fiber products are authentic or counterfeit.

The above checking can be carried out with the naked eye, a magnifying glass, a microscope, etc.

### Effects of the Invention

The invention provides fibers or fiber products wherein the individual yarns can be marked with a minute mark.

The invention also provides a method of producing fibers or fiber products wherein the individual yarns can be marked with a minute mark.

When the fiber or fiber product is irradiated with a laser beam, the irradiated portion changes color, so that marks such as letters, symbols or patterns can be produced on the fiber or fiber product. Since only the portion of the fiber irradiated with a laser beam changes color, individual yarns of the fiber product can be marked with marks, such as letters, symbols, etc.

Brand name products partially or entirely made of the fiber of the invention can be marked with a brand mark or pattern that cannot be distinguished by the naked eye but is distinguishable under a magnifying glass or a microscope, thereby allowing one to easily distinguish whether marketed products are authentic or counterfeit articles, and thus effectively preventing the counterfeiting of brand name products.

The fiber product has the advantage that the product when sold can quickly be marked with the purchaser's name, desired patterns, symbols, etc. in the store.

The fiber or fiber product is expected to find various applications, such as an embroidery substitute.

The basic principle of the present invention will be described below in further detail with reference to the Examples, which are, however, not within the scope of the claims :

### Example 1

A polyester masterbatch (trade name: CESAf LASER NB94120503, product of Clariant International Ltd.) containing 10 wt.% of barium sulfate (mean particle diameter: 1 µm) and 10 wt.% of carbon black was added in an amount of 5 wt.% to a molten polyester (polyethylene terephthalate) prepared by heating to 295°C, so that barium sulfate and carbon black were dispersed in the polyester to give a polyester melt.

The melt was then ejected through a nozzle into the air and the ejected molten filaments were stretched to three times their original length at 115°C, thus giving a polyester fiber (filament yarn, diameter: 100 µm) having barium sulfate and carbon black incorporated therein.

### Example 2

A 6 µm-thick transparent biaxially stretched polyamide film was microslit to a width of 0.2 mm to give slit yarns.

Fibers of the invention having a core-sheath structure were produced by using the barium sulfate-containing polyester fiber (filament yarn) obtained in Example 1 as a core and wrapping the above slit yarn therearound.

### Example 3

The filament yarn obtained in Example 1 was partially irradiated with a Nd-YAG laser (wavelength: 532 nm). In the irradiated portions, phase separation occurred in the carbon black and barium sulfate displayed itself on the surface of the filament yarn. As a result, the portion irradiated with the laser changed from black to white, which was clearly distinguishable with the naked eye from the hue of the portions which had not been irradiated with the laser.

### Example 4

The monofilament yarn obtained in Example 1 was irradiated with a Nd-YAG laser beam (wavelength: 1064 nm) using a scanning laser marking device (product of TAMPOPRINT AG, model number: WS+SK-86) to make alphabetical marks (letter size: 80 µm x 80 µm).

The monofilament yarn was observed under a 200-times optical microscope. The alphabetical marks were clearly recognizable.

## Claims

1. A method of marking a fiber or fiber product with a mark or pattern, comprising irradiating with a laser beam a fiber or fiber product prepared by impregnating an artificial fiber with carbon black and barium sulfate, so that the irradiation causes phase separation of carbon black and allows barium sulfate to clearly appear on the surface of the fiber or fiber product, thereby changing the laser beam-irradiated portion from black to white.

2. The method according to claim 1, wherein the artificial fiber is a polyester.

## Patentansprüche

1. Verfahren zum Markieren einer Faser oder eines Faserprodukts mit einer Markierung oder einem Muster, umfassend das Bestrahlen einer Faser oder eines Faserprodukts, hergestellt durch das Imprägnieren einer künstlichen Faser mit Ruß und Bariumsulfat, mit einem Laserstrahl, so dass die Bestrahlung eine Phasentrennung von Ruß verursacht und es ermöglicht, dass Bariumsulfat auf der Oberfläche der Faser oder des Faserprodukts klar erscheint, wodurch der mit dem Laserstrahl bestrahlte Bereich von schwarz nach weiß wechselt.

2. Verfahren nach Anspruch 1, wobei die künstliche Faser ein Polyester ist.

## Revendications

1. Procédé pour marquer une fibre ou un produit fibreux avec une marque ou un motif, comprenant l'irradiation, avec un faisceau laser, d'une fibre ou d'un produit fibreux préparé par imprégnation d'une fibre artificielle avec du noir de carbone et du sulfate de baryum, de façon que l'irradiation provoque une séparation de phase du noir de carbone et permette au sulfate de baryum d'apparaître clairement sur la surface de la fibre ou du produit fibreux, en faisant ainsi passer du noir au blanc la partie irradiée par le faisceau laser.

2. Procédé selon la revendication 1, dans lequel la fibre artificielle est en polyester.
